

## UNITED STATES PATENT OFFICE

2,623,823

## ENERGIZERS FOR AROMATIC TRIAMINO DEVELOPING AGENTS AND SUPPRESSION OF PROXIMITY DEVELOPMENT IN AZINE COLOR DEVELOPERS

Robert C. Gunther, Galesburg, Ill., assignor to General Aniline &amp; Film Corporation, New York, N. Y., a corporation of Delaware

No Drawing. Application March 21, 1950,  
Serial No. 151,052

12 Claims. (Cl. 95—2)

1

The present invention relates to energizers for aromatic triamino developing agents and to a method of suppressing proximity development in the processing of multilayer color film to azine dyestuff images while employing 2,4-diaminoanilines for color development.

It is known that azine dyestuff images in exposed silver halide emulsions are produced by color developing silver halide emulsions with 2,4-diamino-aniline developing agents in the presence of color formers. The procedure of this process is described in United States Patent 2,486,440, granted on November 1, 1949.

The azine dyes produced in this way have unusual stability and superior spectral characteristics, particularly when compared with the quinonimine or azomethine dyes produced with developers of the p-phenylenediamine type.

Despite the many recognized advantages of this new class of color developers, they possess two disadvantages which provide a somewhat serious problem in the use of the azine method. The first disadvantage occurs in the development of multilayer film and is manifested by a loss of color rendition in the azine images formed in such material.

Such loss of color rendition has been found to be attributable to a phenomenon peculiar to the aforementioned azine processing which is characterized herein as proximity development. The following explanation of such phenomenon will serve to give a better understanding of the objects of the present invention.

As is known, the conventional material employed at the present time in color photography is an integral tripack consisting essentially of three superimposed silver halide emulsion layers, the bottom layer being sensitized to red, the middle layer to green, and the top layer to blue. When such a tripack is exposed, the red densities of the picture are recorded in the bottom layer, the green densities in the middle layer, and the blue densities in the top layer. According to customary practice, the image formed in the respective layers is complimentary in color to the light rays for which the particular layer is sensitized.

One of the best modes of constructing such tripacks involves the utilization in each of the three silver halide emulsion layers of a color former which is rendered non-diffusing in the emulsions. Where such tripacks are of the reversible type, they are processed by developing first in a black and white developer, and finally in a color forming developer.

2

In the color development of such a tripack with a 2,4-diamino-aniline, the color developer reduces in any one layer the silver halide remaining after the first development and is itself oxidized to an active state capable of coupling with the color former present in that layer to form a positive dye image. Consequently, in any one layer the amount of dye produced will be a function of the amount of residual silver halide in that layer and the resulting dye will be formed imagewise. Thus, in each of the three layers of the tripack, one of the primary color densities (blue in the top layer, green in the middle layer, and red in the bottom layer) is accurately recorded in the form of a positive complimentary dye image.

The coupling reaction between the migratory oxidized developer and the immobile color former in each layer is normally rapid so that the oxidized developer travels only a very short distance before encountering the color former molecule and coupling therewith. It often happens, however, that some dye may be produced in a particular layer by the coupling of a color former in that layer with an oxidized developer molecule that originated not in that particular layer but in one of the adjacent layers. Typically, an oxidized developer molecule originating in the red-sensitive layer may escape from this layer without coupling and migrate to the green-sensitive layer to couple with the color former molecule in that layer. As a result, there will be produced in the green-sensitive layer a certain amount of magenta dye which records not the green densities of the original picture, but red densities which should have been confined to the bottom or red-sensitive layer. This migration of oxidized developer from one layer to an adjacent layer is the phenomenon known as proximity development.

The other disadvantage also occurs in the development of multilayer film and is manifested by the inability of the first (black and white) developing agent to reduce the slightly activated silver in the highlight or white portions of the processed film. As a consequence, the highlights of the processed film are not clean, also the color rendition in the lighter densities is somewhat poor. The non-reduction of the slightly activated silver is presumably due to the sluggishness of the first developer.

I have now discovered that this tendency toward proximity development, in the processing of tripacks by the azine method while using 2,4-diamino-aniline for color development, can be eliminated or greatly suppressed by utilizing in

the azine color forming developer, in the concentration of 0.5 to 10 grams per liter, of a reaction product obtained by condensing a 2,4-diamino-aniline with a lower alkyl  $\alpha$ -ketocarboxylic acid or with a lower alkyl aldehyde.

The condensation products are mild black and white developers and are more rapid in their initial reduction of exposed silver halide than the 2,4-diamino-aniline developers. They develop the residual silver halide, present in the highlights, which was not earlier developed due to the sluggishness of the first developer. The slight development in other than highlight density has little noticeable effect on the final image. This development takes place without the formation of color and thus leads to the production of clean whites and brilliant highlights.

The condensation product in the aforesated concentration range energizes the 2,4-diamino-aniline developing agent so that the slightly activated silver is actually reduced. It appears that the reaction product reacts with the slightly activated silver and as a result yields improved color rendition and clean whites due to the development of the slightly activated or residual silver.

When the condensation products are employed in the (reversal) azine developer, the color separation and, consequently, the brilliance of the color images especially the whites are also markedly improved over those obtained, but free from such a reaction product.

The energizing of the 2,4-diamino-aniline developing agent and the suppression of proximity development in the azine procedure while utilizing 2,4-diamino-anilines for color development constitute the purpose and principal object of the present invention.

Other objects and advantages will appear from the following description.

The 2,4-diamino-anilines which are employed as the color developers and for the preparation of the condensation product, by treatment with a lower alkyl  $\alpha$ -ketocarboxylic acid or with lower alkyl aldehyde, are of the type described in the aforementioned Patent No. 2,486,440 and characterized by the following formulae:



and



wherein R<sub>1</sub> is hydrogen or an aliphatic radical, such as alkyl, i. e., methyl, ethyl, propyl, butyl, amyl, and the like, carboxyalkyl, such as carboxymethyl, carboxyethyl, carboxybutyl, and the like, hydroxyalkyl, such as hydroxymethyl, hydroxyethyl, hydroxypropyl, hydroxybutyl, and the like, sulfoalkyl, such as sulfomethyl, sulfo-propyl, sulfobutyl, and the like, R<sub>2</sub> is aliphatic as above, or an aromatic radical, such as aryl, i. e., phenyl, naphthyl, and the like, carboxyaryl, i. e., carboxyphenyl, carboxynaphthyl, and the

70

75

like, sulfoaryl, such as sulfophenyl, sulfonaphthyl, and the like, alkoxyaryl, such as methoxyphenyl, methoxynaphthyl, ethoxyphenyl, butyroxyphephenyl, and the like, alkylaryl, such as toluyl, ethylphenyl, propylphenyl, and the like, heterocyclic, such as 2-pyridyl, 2-piperidyl, 2-indolyl, 2-quinolyl, and the like, R<sub>3</sub> is an aromatic or aliphatic radical as illustrated above, Q represents the atoms necessary to complete a six-membered isocyclic ring system, such as benzo and the like, and Z and Y are hydrogen, sulfo, or carboxy.

The lower alkyl  $\alpha$ -ketocarboxylic acids and lower alkyl aldehydes, which are treated with the 2,4-diamino-aniline to form the condensation product are those of the following formulae:

#### R<sub>4</sub>-CHO and R<sub>5</sub>-COCOOH

wherein R<sub>4</sub> is hydrogen or a lower alkyl, such as methyl, ethyl, propyl, butyl, isobutyl, amyl, and the like, and R<sub>5</sub> is a lower alkyl of the same value as R<sub>4</sub>.

Specific examples of such lower alkyl  $\alpha$ -ketocarboxylic acids and aldehydes are:

25 Pyruvic acid  
 3-methyl-pyruvic acid  
 $\beta$ -ethyl-pyruvic acid  
 $\beta$ -propyl-pyruvic acid  
 $\beta$ -isopropyl-pyruvic acid and the like  
 30 Formaldehyde  
 Acetaldehyde  
 Propionaldehyde  
 Butyraldehyde  
 Isobutyraldehyde, etc.

Specific examples of 2,4-diamino-anilines are:

40 4-( $\beta$ -hydroxyethylamino)-6-(4'-carboxy-methoxy-phenylamino)-metanilic acid  
 4-(carboxymethylamino)-6-(4'-methoxy-phenylamino)-metanilic acid  
 2-( $\beta$ -sulfoethylamino)-4-phenylamino aniline  
 4,6-di( $\beta$ -hydroxyethylamino)-metanilic acid  
 4-( $\beta$ -hydroxyethylamino)-6-phenylamino-metanilic acid  
 45 2-( $\beta$ -hydroxyethylamino)-4-( $\beta$ -sulfoethylamino)-5-methyl aniline  
 4-( $\beta$ -hydroxy- $\beta$ -methyl-ethylamino)-6-phenylamino-metanilic acid  
 4-[ $\alpha$ -di(hydroxyethyl)ethylamino]-6-(3'-ethoxy-phenylamino)-metanilic acid  
 4-( $\beta$ -hydroxyethylamino)-6-methylamino-metanilic acid  
 4-(sulfomethylamino)-6-(methylphenylamino)-metanilic acid.

55 Color formers to be used with the aforesmented developers to give yellow azine dye images are also described in application Serial No. 101,913, filed June 28, 1949, now Patent No. 2,570,116. These compounds are typified by the fact that they are open chain ketomethylene compounds. Examples of such compounds are:

Acetoacetanilide  
 N-1-naphthylacetooacetamide  
 N,N'-ethylenebisacetooacetamide  
 $p,p'$ -bi-o-acetooacetanilide  
 N-2-naphthylbenzoylacetamide  
 $p,p'$ -bi-acetooacetanilide  
 $\alpha,\alpha'$ -terephthaloylbis-(3-chloro-4,6-dimethoxy-acetanilide)  
 $\alpha$ -benzoylacetanilide.

Preferably, the color formers utilized contain a group rendering them non-migratory in the emulsion. Examples of such compounds are:

2-(m-benzoyleacetamidophenyl) - 1 - octadecyl-5-benzimidazolesulfonic acid.

3,3'-ureylenebis - 5 - p - benzoyleacetamidobenzamide-benzenesulfonic acid

2-p-benzoyleacetamidobenzamide- 6 - stearoylamino-p-toluenesulfonic acid

2-(p-benzoyleacetamidophenyl) - 1 - octadecyl-5-benzimidazolesulfonic acid

p-cyanoacetyl-3-octadecenylsuccinalic acid.

10

Color formers capable of producing magenta dyestuff images are also described in application Serial No. 101,913, filed June 28, 1949, as well as in application Serial No. 793,533, filed December 23, 1947, now Patent No. 2,524,741. Preferably, 15 these color formers are 6-halogen-8-hydroxy-quinolines, and particularly those which are non-migratory in the emulsions. Examples of the latter type compounds are:

20 6-stearoylamino-2-(2'-phenyl - 6' - bromo-8'-hydroxy - cinchoninoyl) - aminotoluene-4-sulfonic acid

2-phenyl-6-chloro-8-hydroxy-cinchoninoyl-octadecyl taurine

2-decoxy-3-(2-phenyl-6-bromo-8-hydroxy - cinchoninoyl) - aminobenzenesulfonic acid

2 -(3-stearoylaminophenyl) -6-bromo-8-hydroxy-cinchoninoyl acid

2-stearoylamino-6-(6-chloro-8-hydroxy - cinchoninoyl) -amino-toluene-4-sulfonic acid, and the like.

Color formers for the cyan image are also described in application Serial No. 101,913 and in 35 United States Patent 2,445,252, granted July 13, 1948. Preferably, these color formers are aryl-J-acid derivatives, particularly those containing a group rendering the color former non-migratory in the emulsion. Examples of the latter compounds are:

Dodecyl urethane of  $\beta$ -sulfoethyl-J-acid

Tetradecyl urethane of p-anisyl-J-acid

2-hexadecyl urethane of phenyl-J-acid

4-stearoylaminophenyl-J-acid, and the like.

The reaction products of 2,4-diamino-anilines with the lower alkyl  $\alpha$ -ketocarboxylic acid or aldehyde utilized in accordance with the present invention are prepared by first suspending one part of a 2,4-diamino-aniline in a mixture of 2.5 parts of a lower boiling alcohol, such as methyl, ethyl, or isopropyl alcohol, in 1 part of 3N hydrochloric acid solution. To this mixture 3 parts of either the acid or aldehyde are added and the whole warmed on a steam bath to 40-50° C. until the solution of the 2,4-diamino-aniline is completed. This usually takes about 10 to 15 minutes. The clear, amber-colored solution is treated with decolorizing carbon and filtered. The hot filtrate is diluted with 3 parts of alcohol and cooled in an ice bath. The product, which separates as pink to colorless crystals, is collected on a Buchner funnel, washed with alcohol, and dried. The yield of the final product is in the range of 60-70%.

Although the exact composition of the reaction product has not been definitely established, it is believed to be of the dihydrobenzimidazole type. The formation of such a compound might be postulated on the basis of the following reaction while utilizing 4 - ( $\beta$  - hydroxyethylamino) - 6 - phenylamino-metanilic acid as the 2,4-diamino-aniline and (1) 3-methyl-pyruvic acid as the 70

lower alkyl  $\alpha$ -ketocarboxylic acid and (2) propionaldehyde as the aldehyde:



10

6



20



30

40

50

The reaction products, prepared in accordance with the foregoing procedure and more fully described in my application Serial No. 151,053, filed on March 21, 1950, are added to azine color developers that are used for the development by diffusion where the color forming component is in solution in the color developer, or development of emulsions containing non-diffusing color formers, and development by either reversal or negative processing procedures.

The following examples describe in detail 45 methods for accomplishing the above objects, but it is to be understood that they are inserted merely for purposes of illustration and are not to be construed as limiting the scope of the invention.

#### Example I

A 4" x 5" sheet of an integral tripack composed of a red-sensitive bottom layer containing a non-diffusing azine cyan dye forming color component, a green-sensitive middle layer containing a non-diffusing azine magenta dye forming color component, and a blue-sensitive top layer containing a non-diffusing azine yellow dye forming color component, was exposed and the latent image developed for 10 minutes at 68° F. in a black and white developer of the following composition:

|                                  |    |      |
|----------------------------------|----|------|
| p-Monomethylamino phenol sulfate | g  | 2    |
| Sodium sulfite                   | g  | 20   |
| Hydroquinone                     | g  | 4    |
| Sodium carbonate                 | g  | 80   |
| Sodium thiocyanate               | g  | 5    |
| Potassium bromide                | g  | 4    |
| Water to make                    | cc | 1000 |

The developed film was shortstopped for 3 minutes in a 3% aqueous solution of acetic acid, re-exposed and color developed for 15 minutes at 68° F. in a developer of the following composition:

|                                                  |    |      |
|--------------------------------------------------|----|------|
| 4-( $\beta$ -hydroxyethylamino)-6-allyl - amino- |    |      |
| metanilic acid                                   | g  | 6    |
| Sodium carbonate, monohydrate                    | g  | 40   |
| Sodium sulfite                                   | g  | 60   |
| Potassium bromide                                | g  | 7.5  |
| Pyridine                                         | g  | 12   |
| Reaction product from 4-( $\beta$ -hydroxy-      |    |      |
| ethylamino - 6 - phenylamino - metanil-          |    |      |
| ic acid and pyruvic acid                         | g  | 3    |
| Water to make                                    | cc | 1000 |

After development, the color developed film was bleached in a ferricyanide bleach bath, fixed in an acid hardening hypo bath, and bathed for a few minutes in a bicarbonate-formaldehyde hardening bath.

After drying, the film showed much better color rendition and cleaner whites. In fact, the blues, greens, and reds of the film were substantially more brilliant than those in the same film developed in the same color developer but not containing the reaction product from 4-methylamino-6-phenylamino-metanilic acid and pyruvic acid.

*Example II*

A developer solution of the following composition was prepared:

|                                                  |    |      |
|--------------------------------------------------|----|------|
| 4 - ( $\beta$ - hydroxyethylamino) - 6 - phenyl- | g  | 5    |
| amino-metanilic acid                             | g  |      |
| Sodium carbonate, monohydrate                    | g  | 50   |
| Sodium sulfite                                   | g  | 50   |
| Potassium bromide                                | g  | 4.5  |
| Benzylamine                                      | g  | 10   |
| Reaction product from 4 - ( $\beta$ - hydroxy-   |    |      |
| ethylamino - 6 - phenylamino - metanil-          |    |      |
| ic acid and $\beta$ -ethyl-pyruvic acid          | g  | 2.5  |
| Water to make                                    | cc | 1000 |

An integral tripack composed of a red-sensitive bottom layer containing a cyan color 40 former,



a green-sensitive middle layer containing a magenta color former.



and a blue-sensitive top layer containing a yellow color former.



was exposed, the latent image developed in a black and white developer as in Example I, re-exposed, and then developed for 15 minutes in the above developer solution.

After development, the film was washed, 75

bleached in ferricyanide bleach, and fixed in an acid hardening hypo solution.

As a result, there was obtained a multicolor positive (cyan dye in bottom, magenta in middle, and yellow in top) of exceptional clarity and brilliance, with unusually clean whites.

*Example III*

An integral tripack with a bottom layer composed of a red-sensitive emulsion containing phenyl-J-acid-octadecyl urethane, a middle layer composed of a green-sensitive emulsion containing 2 - stearoylamino-6-(8-hydroxycinchoninoylamino)-toluene-4-sulfonic acid, and a top layer composed of a blue-sensitive emulsion containing 2 - (4 - benzoylacetaminophenyl) - 1 - octadecyl-5-benzimidazole sulfonic acid was exposed and the latent image developed in a black and white developer, re-exposed, and the residual silver halide developed in a solution of the following composition:

|                                                |    |      |
|------------------------------------------------|----|------|
| 4-( $\beta$ - hydroxyethylamino) - 6 - phenyl- | g  | 5    |
| amino-metanilic acid                           | g  |      |
| Sodium carbonate, monohydrate                  | g  | 40   |
| Sodium sulfite                                 | g  | 60   |
| Potassium bromide                              | g  | 5    |
| Pyridine                                       | g  | 16   |
| Benzylamine                                    | g  | 1    |
| Reaction product from 4-methylamino-6-         |    |      |
| phenylamino-metanilic acid and pro-            |    |      |
| pionaldehyde                                   | g  | 4    |
| Water to make                                  | cc | 1000 |

After development, the film was washed, bleached in a ferricyanide bleach, fixed in an acid hardening hypo, and bathed in a bicarbonate-formaldehyde hardening bath. There was thus obtained a film in which the blues, greens, and reds were substantially more brilliant than those in the same film developed in the same color developer but not containing the reaction product from 4-methylamino-6-phenylamino-metanilic acid and propionaldehyde.

*Example IV*

Example II was repeated with the exception that the reaction product from 4-( $\beta$ -hydroxyethylamino)-6-phenylamino-metanilic acid and  $\beta$ -ethyl-pyruvic acid was replaced by the same quantity of the reaction product from 4-methylamino-6-phenylamino-metanilic acid and acetaldehyde.

*Example V*

Example III was repeated with the exception that the reaction product from 4-methylamino-6-phenylamino-metanilic acid and propionaldehyde was replaced by 3 grams of the reaction product from 4-( $\beta$ -hydroxyethylamino)-6-phenylamino-metanilic acid and 3-methyl-pyruvic acid.

I claim:

1. A photographic developer comprising a 2,4-diamino-aniline and a product obtained by the condensation reaction of a 2,4-diamino-aniline with a compound selected from the class consisting of the following formulas:



70 with elimination of water, wherein  $R_4$  is selected from the class consisting of hydrogen and lower alkyl, and  $R_5$  is lower alkyl.

2. A developer according to claim 1, in which the condensation reaction product is that from 4-( $\beta$ -hydroxyethylamino)-6-phenyl-amino-meth-anilic acid and pyruvic acid.

3. A developer according to claim 1, in which the condensation reaction product is that from 4- $\beta$ -hydroxyethylamino) - 6 - phenylamino - metanilic acid and acetaldehyde.

4. A developer according to claim 1, in which the condensation reaction product is that from 4-methylamino - 6 - phenylamino-metanilic acid and propionaldehyde.

5. A developer according to claim 1, in which the condensation reaction product is that from 4 - methylamino-6-phenylamino-metanilic acid and  $\beta$ -ethyl-pyruvic acid.

6. A developer according to claim 1, in which the condensation reaction product is that from 4-( $\beta$ -hydroxyethylamino)-6-phenylamino - metanilic acid and 3-methyl-pyruvic acid.

7. In the process of producing subtractively colored azine dye images in a tripack consisting of three superimposed silver halide emulsion layers containing color formers capable of coupling with the oxidation products of a 2,4-diamino-aniline developing agent to form azine dye images by exposing and developing the same with a color developer containing as the effective developing agent 2,4-diamino-aniline, the improvement wherein said developer additionally contains a product obtained by the condensation reaction of 2,4-diamino-aniline with a compound selected from the class consisting of the following formulae:

30 R<sub>4</sub>-CHO and R<sub>5</sub>-COCOOH

with the elimination of water wherein R<sub>4</sub> is selected from the class consisting of hydrogen and lower alkyl, and R<sub>5</sub> is lower alkyl.

8. The process as defined in claim 7, wherein 35

the condensation reaction product contained in the color developer is that from 4-( $\beta$ -hydroxyethylamino)-6-phenylamino-metanilic acid and pyruvic acid.

9. The process as defined in claim 7, wherein the condensation reaction product contained in the color developer is that from 4-( $\beta$ -hydroxyethylamino)-6-phenylamino-metanilic acid and acetaldehyde.

10. The process as defined in claim 7, wherein the condensation reaction product contained in the color developer is that from 4-methylamino-6-phenylamino-metanilic acid and propionaldehyde.

11. The process as defined in claim 7, wherein the condensation reaction product contained in the color developer is that from 4-methylamino-6-phenylamino-metanilic acid and  $\beta$ -ethyl-pyruvic acid.

12. The process as defined in claim 7, wherein the condensation reaction product contained in the color developer is that from 4( $\beta$ -hydroxyethylamino)-6-phenylamino-metanilic acid and 3-methyl-pyruvic acid.

ROBERT C. GUNTHER.

#### REFERENCES CITED

The following references are of record in the file of this patent:

#### UNITED STATES PATENTS

| Number    | Name     | Date         |
|-----------|----------|--------------|
| 2,440,954 | Jennings | May 4, 1948  |
| 2,486,440 | Schmidt  | Nov. 1, 1949 |